

## UNITED STATES PATENT OFFICE

1,982,381

METHOD OF MAKING A MATERIAL FOR USE  
IN CAULKING, PACKING, LAGGING, OR  
COVERING, AND FOR OTHER PURPOSESEugene Victor Hayes-Gratze, Kensington,  
London, EnglandNo Drawing. Original application March 7, 1933,  
Serial No. 659,984. Divided and this applica-  
tion August 23, 1933, Serial No. 686,442. In  
Great Britain March 12, 1932

## 2 Claims. (Cl. 28—1)

This invention relates to caulking, packing, lagging or covering and reinforcing material for use in making pipe and other joints, for jacketing, lagging and insulating pipes, tanks and the like, for use in brake linings, floor coverings, moulded india rubber reinforcements, cable coverings, hose pipes, shoe soles and other purposes, in many of which cotton, flax or like vegetable fibres or animal fibres are at present employed.

5 This application is a division of my copending application, Ser. No. 659,984, filed Mar. 7, 1933.

The primary object of the present invention is the production of an inexpensive hard wearing material for a variety of purposes in which resistance to decay and unaffectedness at relatively high temperatures are of importance.

The present invention comprises the use of vegetable fibres carded, spun and woven into a material, treated with any suitable binding, 20 plastic, protective or lubricating material and with or without a suitable filling material and formed into a material which is most readily used for its intended purpose.

In one embodiment of this invention, particularly adapted for use in caulking or packing the joints or flanges of pipes, or for use as a lagging or jacketing for pipes, tanks and the like, vegetable fibres such as sisal, hemp, or preferably coir or coco-nut fibre after extraction and in their 25 natural state after extraction, which process is one in which the fibres are softened or entirely de-gummed by treatment with a neutralized sulphonated oil treated to an electric ionization process as described in my prior U. S. Patent No. 35 1,913,202 dated the 6th of June 1933, are combed, carded, spun and woven so as to produce a textile material. This textile material is then incorporated with any suitable binding, plastic, protective or lubricating material, for instance oil, 40 bitumen, sodium or potassium silicate, calcium sulphate, alum or aluminium acetate, cement, gums, india rubber, powdered talc or plumbago. Such materials may be dissolved or mixed with 45 any suitable liquid, into which the textile material is immersed, sprayed or otherwise treated, or alternatively the materials may be incorporated with the material in a dry state and subsequently treated with a liquid or solvent. After 50 such treatment, the treated material may be rolled or pressed to exclude excess liquid and subjected to a heat treatment or vulcanization to mould it to a shape or form according to its intended use. In some cases a suitable filling material, such as cork or the fleshy matter from which 55 vegetable fibres have been extracted, for example

the pith surrounding coir, may also be incorporated with the fibrous mass before or after weaving.

It has been found that a material in which the basic component is softened coir, not only forms a highly resilient packing unaffected by compression or by fluids, even superheated steam, but also an efficient lagging for pipes and containers for insulating them from heat losses and is moreover very resistant to disintegration.

A woven material in which the basic material is softened coir can be usefully employed as a backing or cloth for floor coverings, for example linoleum, floor cloth and the like, and for such purposes has definite advantages over the usual hemp or jute backings at present employed.

The vegetable fibres—preferably coir—are extracted or treated and softened by means of a reagent (or an aqueous solution thereof) prepared by treating a neutralized sulphonated oil to an electric ionization and/or ozonization process. Coir so treated may be readily spun and woven into a relatively fine material which may be coated or impregnated with raw india rubber or india rubber mixture and afterwards vulcanized by heat.

In a further modification, the treated fibrous material may be woven or braided to envelop a metal core of one or more strands of wire, alone or in combination with a mass of the unspun vegetable fibres. The product may be impregnated or compounded with a suitable binding, protective, filling or lubricating material as hereinbefore described.

I declare that what I claim and desire to secure by Letters Patent is:—

1. A method of producing a material for use in caulking, packing, lagging or covering and for other purposes, consisting firstly in softening natural vegetable fibres and making them permeable to an agglutinating material by treating them with a reagent prepared by treating a neutralized sulphonated oil to an electric ionization process, secondly; carding the softened fibres, thirdly; spinning the fibres into yarn, fourthly; weaving the yarn to produce a textile material, fifthly; immersing the textile material in a solution of agglutinating material, sixthly; compressing the material to exclude surplus solution and to mould it to shape according to its intended use, as set forth.

2. A method of producing a material for use in caulking, packing, lagging or covering and for other purposes, consisting firstly in softening coir and making it permeable to an agglutinating

material by treating it with a reagent prepared by  
treating a neutralized sulphonated oil to an elec-  
tric ionization process, secondly; carding the  
softened coir, thirdly; spinning the softened coir  
5 into yarn, fourthly; weaving the yarn to produce

a textile material, fifthly; immersing the woven  
material in a bituminous solution, sixthly; rolling  
the treated material to remove excess solution, to  
compress it and to reduce its bulk, as set forth.

EUGENE VICTOR HAYES-GRATZE.

80

10

85

15

90

20

95

25

100

30

105

35

110

40

115

45

120

50

125

55

130

60

135

65

140

70

145

75

150